

## 1

3,535,251

### ACRYLONITRILE POLYMERS PLASTICIZED WITH PHENOLIC ESTERS OF ALKYL SULPHONIC ACIDS

Wilhelm Brenschede, Herbert Marzolph, and Alfred Nogaj, Dormagen, Helmut Reichardt, Dormagen-Horrem, and Alfred Reichle and Martin Wandel, Dormagen, Germany, assignors to Farbenfabriken Bayer Aktiengesellschaft, Leverkusen, Germany, a corporation of Germany

No Drawing. Filed Sept. 2, 1966, Ser. No. 576,815  
Claims priority, application Germany, Sept. 11, 1965,  
F 47,165, F 47,166, F 47,167  
Int. Cl. C08f 45/46; C08k 1/54

U.S. CL. 260—30.8

3 Claims

#### ABSTRACT OF THE DISCLOSURE

Acrylonitrile polymers in filament, fibre, or film form having improved mechanical properties and containing as a plasticiser

- (a) aryl ester of an alkyl sulphonic acid having 6 to 18 carbon atoms in the alkyl group;
- (b) mixtures of lower alkyl phthalate esters and the above sulphonic acid esters; or
- (c) mixtures of lower alkyl phthalate and polyester of adipic acid.

This invention relates to a process for the production of filaments, fibres and films from acrylonitrile polymers in which the mechanical properties of the filaments, fibres and films are improved by the addition of plasticisers.

Numerous compounds have already been proposed as being suitable for use as plasticisers for polyacrylonitrile. For example, cyanoalkyl-sulphonamides, dioxanones, phthalic acid esters, polynitrile compounds and phosphine compounds, have been described as plasticisers for polyacrylonitrile. Plasticisers of this kind are added in quantities of 1 to 50% by weight, depending upon the purpose for which the polymer is to be used. They may act either as permanent or as temporary plasticisers. In the production of filaments, fibres and films, plasticisers can only be added in a specific concentration range which is governed both by the particular type of addition and by the substrate. If the plasticiser is added in too large a quantity, the mechanical and thermal properties are unfavourably influenced. If, on the other hand, it is added in too small a quantity, it will not produce the required improvement in the permanent properties, such as the permanent flexural index and flexural abrasion resistance etc. The optimal concentration for the particular circumstances can readily be determined by experiment.

A process for the production of filaments, fibres and films with improved mechanical properties from acrylonitrile polymers has now been found, in which 1 to 20% either of an alkylsulphonic acid aryl ester having 6 to 18 carbon atoms in the alkyl group or of a mixture of an alkyl phthalate having 1 to 4 carbon atoms in each of the alkyl groups, with an alkyl sulphonic acid ester or a polymeric adipic acid ester, is added to the acrylonitrile polymers, which are then further processed to form filaments, fibres and films.

An example of a suitable alkyl phthalate having 1 to 4 carbon atoms in the alkyl groups is dimethyl phthalate. Polymeric esters of adipic acid and aliphatic diols with 2 to 8 carbon atoms, preferably butane diol or hexane diol, may be used as the polymeric adipates. The molecular weights of the polymeric adipates are advantageously from 1000 to 3500. Preferred alkyl sulphonic acid aryl

## 2

esters are those which have been prepared from a mixture of phenol and cresol.

The filaments, fibres and films produced by the process according to the invention from acrylonitrile polymers, are distinguished from polyacrylonitrile films or materials which do not contain the plasticisers in the concentration range specified, by the fact that they exhibit significantly improved permanent properties (flexural and abrasion resistance indices), whilst their other technological properties show little or no change. It was discovered, surprisingly so, that, for example, their tensile strength is not only retained but, in fact, shows some improvement in the case of films. There is little or no increase in breaking elongation. In the case of films, the high brittleness and tendency to split or crack of a polyacrylonitrile film without any additives, can often give the impression of an increase in breaking elongation. The softening range of the filaments, fibres and films is not affected by the addition of the plasticisers used according to the present invention. It is also remarkable that the films in particular, but also the filaments and fibres produced in accordance with the present invention, show a greatly reduced tendency to split and fibrillate.

In order to produce filaments, fibres or films from acrylonitrile polymers in the presence of the plasticiser, an ester of an alkyl sulphonic acid and phenols or cresols may be added to the solutions of polyacrylonitrile in solvents such as dimethyl formamide, dimethyl acetamide and dimethyl sulphone, used to produce the filaments, fibres or films, after which these solutions are further processed by known methods to form the films, filaments or fibres.

It is also possible to make the acrylonitrile polymer into a paste with the plasticisers, before dissolution.

In the context of the present invention, filaments, fibres or films of acrylonitrile polymers also include structures of the same kind consisting of copolymers of acrylonitrile with other polymerisable monomers or of mixtures of these copolymers or of polyacrylonitrile with other polymers, providing the amount of acrylonitrile component is at least 80% by weight.

#### EXAMPLE 1

16% by weight based on polymer of a sulphonic acid ester, were added to a polyacrylonitrile spinning solution in dimethyl formamide containing 25% by weight of a copolymer of 95% by weight of acrylonitrile and 5% by weight of methyl acrylate. The sulphonic acid ester was the product of an aliphatic C<sub>15</sub>-acid and a mixture of equal parts of phenol and cresol. The solution was spun in the usual way by the dry spinning method, stretched and fixed. The completed fibres had an individual denier of 15 and a residual dimethyl formamide content of approximately 1.5% by weight. For comparison purposes, an identical solution was spun and further processed in the same way, in the absence of the sulphonic acid ester.

The properties of the fibres are set out in Table 1 below.

The permanent flexural index (number of folds or bends before failure) was measured on a "Zweigle" permanent flexure testing machine. It was enlarged to include ten measuring points, and the bending edge adapted to the testing denier of 15 den. During each test, the filament was subjected to a load equivalent to 10% of the tenacity.

The remaining technological properties were tested in accordance with the appropriate DIN specifications. The "softening range" was determined by measuring the

tensile strain under heat at a load of 1.0 p./tex and a temperature increase of 1° C. per minute.

TABLE 1

| Mechanical properties                                              | Fibre with plasticiser of Example 1 | Fibre without plasticiser |
|--------------------------------------------------------------------|-------------------------------------|---------------------------|
| Average permanent flexural index (double bends)                    | 18,600                              | 6,200                     |
| Average wire abrasion index (double strokes)                       | 6,900                               | 3,200                     |
| Tenacity, p./den.                                                  | 1.23                                | 1.27                      |
| Breaking elongation, percent                                       | 79                                  | 91                        |
| Relative loop tenacity                                             | 85                                  | 92                        |
| Initial E-modulus, kp./mm <sup>2</sup>                             | 219                                 | 260                       |
| Elastic recovery elongation (3 mins. load—3 mins. recovery period) | 64                                  | 67                        |
| Softening temperature, °C                                          | 95-100                              | 94-98                     |

## EXAMPLE 2

16% by weight based on polymer, of a sulphonic acid ester were added to a polyacrylonitrile spinning solution in dimethyl formamide containing 25% by weight of a copolymer of 95% by weight acrylonitrile and 5% by weight of methyl acrylate. The sulphonic acid ester was the product of a mixture of aliphatic acids with an average of 11 carbon atoms, and a mixture of equal parts of phenol and cresol. The solution was spun in the usual way by the dry-spinning method, stretched and fixed. The completed fibres had an individual denier of 15 den. and a residual dimethyl formamide content of approximately 1.5% by weight. For comparison, an identical solution was spun and further processed in the same way in the absence of sulphonic acid ester.

The properties of the fibres are set out in Table 2 below.

The permanent flexural index (number of folds before failure) was determined on a "Zweigle" permanent flexure testing machine which had been enlarged to include 10 measuring points and the bending edge adapted to the testing denier of 15 denier. During each test, the load exerted on the filaments amounted to 10% of the tenacity. The bending edge of the permanent flexure tester used for this example had been provided with a smaller radius of curvature than had been used in Example 1.

This modification was made in order to obtain shorter testing times. The other technological properties were measured in accordance with the corresponding DIN specifications.

TABLE 2

| Mechanical properties                                             | Fibre with plasticiser of Example 2 | Fibre without plasticiser |
|-------------------------------------------------------------------|-------------------------------------|---------------------------|
| Average permanent flexure index (double bonds)                    | 10,285                              | 1,450                     |
| Tenacity, p./den.                                                 | 1.10                                | 1.35                      |
| Breaking elongation, percent                                      | 47                                  | 55                        |
| Elastic recovery at 5% elongation (3 mins. load—3 mins. recovery) | 72                                  | 67                        |

## EXAMPLE 3

8% by weight based on polymer, of a sulphonic acid ester were added to a polyacrylonitrile spinning solution in dimethyl formamide containing 25% by weight of a copolymer of 95% by weight of acrylonitrile and 5% by weight of methyl acrylate. The sulphonic acid ester was the product of a mixture of aliphatic acids with an average of 11 carbon atoms, and a mixture of equal parts of phenol and cresol.

Films approximately 30 $\mu$  thick were drawn on a casting drum. The films were stretched 1:3.5 over an edge heated at 150° C., washed with hot water and tempered for 10 minutes at 140° C. They were then 12 $\mu$  thick and had a residual dimethyl formamide content of approximately 1.5% by weight. For comparison, a film was similarly prepared in the absence of a sulphonic acid ester.

The properties set out in Table 3 were measured on these films: Permanent flexural index according to DIN

53374 at 10% of the tenacity: tenacity and breaking elongation according to DIN 53371.

TABLE 3

| 5                               | Fibre with plasticiser of Example 3 | Fibre without plasticiser |
|---------------------------------|-------------------------------------|---------------------------|
| Average permanent flexure index | 6,900                               | 2,50                      |
| Tenacity, kp./mm <sup>2</sup>   | 13.2                                | 13.9                      |
| Breaking elongation, percent    | 10.0                                | 10.9                      |

## EXAMPLE 4

2% by weight of dimethyl phthalate and 2% by weight of a sulphonic acid ester, based on polymer, were added to a polyacrylonitrile spinning solution in dimethyl formamide containing 25% by weight of a copolymer of 95% by weight of acrylonitrile and 5% by weight of methyl acrylate.

The sulphonic acid ester was the product of an aliphatic C<sub>15</sub>-acid and a mixture of equal parts of phenol and cresol. The solution was spun in the usual way by the dry spinning process, stretched and fixed. The completed fibres had an individual denier of 15 den. and a residual dimethyl formamide content of 1.5% by weight. For comparison, an identical solution was spun and further processed in the same way in the absence of dimethyl phthalate and sulphonic acid ester.

The properties of the fibres are set out in Table 4 below.

The permanent flexural index (number of folds before failure) was determined on a "Zweigle" permanent flexure testing machine which had been enlarged to include 10 measuring points, and the bending edge adapted to the testing denier of 15 den. The load placed on the filaments during each test amounted to 10% of the tenacity.

The wire abrasion index was determined by Grunewald's method (Chemiefasern, 1963, p. 853 et seq.) under a load of 1 g. The other technological properties were measured in accordance with the appropriate DIN specifications. The tensile strain under heat was measured at a load of 1.0 p./tex at a temperature increase of 1° C. per minute in order to determine the "softening range."

TABLE 4

| 45                                                                                    | Fibre with plasticiser of Example 4 | Fibre without plasticiser |
|---------------------------------------------------------------------------------------|-------------------------------------|---------------------------|
| Average permanent flexure index (double bonds)                                        | 32,500                              | 6,200                     |
| Average wire abrasion index (double strokes)                                          | 10,300                              | 3,200                     |
| Tenacity, p./den.                                                                     | 1.00                                | 1.27                      |
| Breaking elongation, percent                                                          | 96                                  | 91                        |
| Rel. loop tenacity, percent                                                           | 100                                 | 92                        |
| Initial E-modulus, kp./mm <sup>2</sup>                                                | 294                                 | 260                       |
| Torsion modulus, kp./mm <sup>2</sup>                                                  | 145                                 | 147                       |
| Elastic recovery at 5% elongation, percent (3 mins. load and 3 mins. recovery period) | 69                                  | 67                        |
| Softening temperature, °C                                                             | 96-100                              | 94-98                     |

## EXAMPLE 5

8% by weight of dimethyl phthalate and 8% by weight of a sulphonic acid ester, based on polymer, were added to a polyacrylonitrile spinning solution in dimethyl formamide containing 25% by weight of a copolymer of 95% by weight of acrylonitrile and 5% by weight of methyl acrylate. The sulphonic acid ester was the product of a mixture of aliphatic acids with an average of 11 carbon atoms, and a mixture of equal parts of phenol and cresol.

The solution was spun in the usual way by the dry spinning process, stretched and fixed. The finished fibres had an individual denier of 15 den. and a residual dimethyl formamide content of approximately 11.5% by weight.

For comparison, an identical solution was spun and further processed in the same way in the absence of dimethyl phthalate and sulphonic acid ester.

The properties of the fibres are set out in Table 5 below.

The permanent flexural index (number of folds before failure) was determined on a "Zweigle" permanent flex-

ure testing machine which had been enlarged to include 10 measuring points, and the bending edge adapted to the testing denier of 15 den. The bending edges of this machine had been provided with a smaller radius of curvature than had been used in Example 1. The object of this was to shorten the testing time. The load placed on the filament during each test amounted to 10% of the tenacity.

The other technological properties were measured in accordance with the corresponding DIN specifications.

TABLE 5

| Mechanical properties                                                                 | Fibre with plasticiser of Example 5 | Fibre without plasticiser |
|---------------------------------------------------------------------------------------|-------------------------------------|---------------------------|
| Permanent repeated flexure index (double bends)-----                                  | 9,780                               | 1,450                     |
| Tenacity, p./den-----                                                                 | 1.01                                | 1.35                      |
| Breaking elongation, percent-----                                                     | 41                                  | 55                        |
| Elastic recovery at 5% elongation, percent (3 mins.' load and 3 mins.' recovery)----- | 76                                  | 67                        |

## EXAMPLE 6

A mixture of 4% by weight of dimethyl phthalate and 4% by weight of a sulphonic acid ester, based on polymer, was added to a polyacrylonitrile spinning solution in dimethyl formamide containing 25% by weight of a copolymer of 95% by weight of acrylonitrile and 5% by weight of methyl acrylate.

The sulphonic acid ester was the product of a mixture of aliphatic acids with an average of 11 carbon atoms, with a mixture of equal parts of phenol and cresol. Films approx. 30 $\mu$  thick were drawn on a casting drum. The films were then stretched 1:3.5 over and edge heated at 150° C., washed with hot water and tempered for 10 mins. at 140° C. The film was then 12 $\mu$  thick and had a residual dimethyl formamide content of approximately 1.5% by weight. For comparison, a film was produced in the same way in the absence of the aforementioned plasticiser-like mixture.

The properties set out in Table 6 were determined on these films:

Repeated flexural index according to DIN 53374 at 10% of the breaking load; breaking elongation and tenacity according to DIN 53371:

TABLE 6

|                                       | Film with plasticiser of Example 6 | Film without plasticiser |
|---------------------------------------|------------------------------------|--------------------------|
| Permanent repeated flexure index----- | 6,200                              | 2,500                    |
| Tenacity, kp./mm. <sup>2</sup> -----  | 15.5                               | 13.9                     |
| Breaking elongation, percent-----     | 18.3                               | 10.9                     |

## EXAMPLE 7

A mixture of 8% by weight of a polyadipate and 8% by weight of dimethyl phthalate, based on polymer, was added to a polyacrylonitrile spinning solution in dimethyl formamide containing 25% by weight of a copolymer of 95% by weight of acrylonitrile and 5% by weight of methyl acrylate. The polyadipate had an average molecular weight of 2000 to 2500. It had been prepared from 66 parts by weight of adipic acid, 32 parts by weight of hexane diol and 22 parts by weight of butane diol.

The solution was spun in the usual way by the dry spinning process, stretched and fixed. The completed fibres had an individual denier of 15 and a residual dimethyl formamide content of approximately 1.5% by weight. For comparison, an identical solution was spun and fur-

ther processed in the same way in the absence of the plasticiser mixture.

The properties of the fibres are set out in Table 7 below.

The permanent flexural index (number of folds before failure) was determined on a "Zweigle" permanent flexure testing machine which had been enlarged to include 10 measuring points, and the bending edge adapted to the testing denier of 15. The load placed on the filament amounted to 10% of the tenacity. The wire abrasion index was determined by Grunewald's method (cf. *Chemiefasern*, 1963, pp. 853 et seq.) at a load of 1 g. The tensile strain under heat was determined at a load of 1.0 p./tex and a temperature increase of 1° per minute in order to determine the softening range. The other technological properties were tested in accordance with the corresponding DIN specifications:

TABLE 7

|                                                                                 | Fibre with plasticiser of Example 7 | Fibre without plasticiser |
|---------------------------------------------------------------------------------|-------------------------------------|---------------------------|
| Permanent repeated flexure index (double bends)-----                            | 21,300                              | 6,200                     |
| Average wire abrasion index (double strokes)-----                               | 7,200                               | 3,200                     |
| Tenacity, p./d.-----                                                            | 0.90                                | 1.27                      |
| Breaking elongation, percent-----                                               | 113                                 | 91                        |
| Rel. loop tenacity, percent-----                                                | 87                                  | 92                        |
| Initial E-modulus, kp./mm. <sup>2</sup> -----                                   | 162                                 | 260                       |
| Elastic recovery at 5% elongation (3 mins.' load—3 mins.' recovery period)----- | 65                                  | 67                        |
| Softening range, ° C.-----                                                      | 88-91                               | 94-96                     |

What we claim is:

1. A plasticized acrylonitrile polymer comprising a mixture of an acrylonitrile polymer containing at least 80% by weight of polymerized acrylonitrile and up to 20% by weight of methyl acrylate and 1 to 20% by weight of the acrylonitrile polymer of a plasticizer selected from the group consisting of phenolic, cresolic, and mixed phenolic and cresolic esters of alkyl sulphonic acids, wherein the alkyl radical has from 6 to 18 carbon atoms.

2. The plasticized acrylonitrile polymer of claim 1 wherein the polymer is a copolymer comprising 80 to 95% by weight of acrylonitrile and 20 to 5% by weight of methyl acrylate.

3. The plasticized polymer of claim 2 wherein the copolymer comprises 95% by weight of acrylonitrile and 5% by weight of methyl acrylate.

## References Cited

## UNITED STATES PATENTS

|              |         |                        |          |
|--------------|---------|------------------------|----------|
| 2,404,717    | 7/1946  | Houtz -----            | 260—30.8 |
| 2,426,728    | 9/1947  | D'Alieio.              | 260—30.8 |
| 2,474,350    | 6/1949  | Eilerman -----         | 260—30.8 |
| 2,503,245    | 4/1950  | Coover et al. -----    | 260—30.8 |
| 55 2,555,062 | 5/1951  | Small et al. -----     | 260—31.6 |
| 2,559,172    | 7/1951  | Schneider et al. ----- | 260—32.4 |
| 2,689,862    | 9/1954  | Knowles -----          | 260—30.8 |
| 3,053,789    | 9/1962  | De Witt -----          | 260—30.8 |
| 3,328,365    | 6/1967  | Aubrey et al. -----    | 260—31.8 |
| 2,613,195    | 10/1952 | Craig -----            | 260—30.8 |
| 2,474,350    | 6/1949  | Eilerman -----         | 260—30.8 |

MORRIS LIEBMAN, Primary Examiner

P. R. MICHL, Assistant Examiner

U.S. CL. X.R.

260—31.6, 31.8